

## UNITED STATES PATENT OFFICE

1,922,033

## TREATMENT OF TEXTILE MATERIALS

George Holland Ellis and William Bertram Miller, Spondon, near Derby, England, assignors to Celanese Corporation of America, a Corporation of Delaware

No Drawing. Application August 6, 1929, Serial No. 383,977, and in Great Britain August 24, 1928

11 Claims. (Cl. 8—5)

The colouration of textile materials can be effected, as is known, by the oxidation thereon of various oxidizable aromatic compounds, for example, aromatic bases such as p-amino-di-5 phenylamine,  $\alpha$ -naphthylamine, benzidine, or aniline, or mixtures thereof. In producing such colourations the material is usually padded or otherwise treated with a solution containing the aromatic compound and an oxidizing agent, the 10 action of the latter being promoted by a subsequent ageing process.

Difficulties have been experienced in the production of "resist" effects under such colourations by printing the material, after impregnating with the aromatic compound and oxidizing agent, with an alkali or a reducing agent to inhibit the action of the oxidizing agent on selected areas during a subsequent ageing or steaming process. Oxidation of the aromatic compound 20 tends to occur prior to the application of the alkali or reducing agent with the result that the "resisted" portions are liable to be stained by the oxidation products.

It has been found that this tendency can be 25 very much diminished or entirely avoided and that purer white or coloured "resist" effects can be produced with oxidation colourations on textile materials, and more particularly on materials made of or containing cellulose esters, for 30 example cellulose acetate, or cellulose ethers, by ensuring that the oxidizable aromatic compound and oxidizing agent are never, even prior to the ageing process, present simultaneously on the parts of the material which are not to be coloured 35 by the oxidation products of the oxidizable compounds.

According to the present invention therefore pattern effects are produced by the formation of oxidation colourations on materials, particularly 40 materials made of or containing cellulose acetate or other cellulose esters or ethers, by a process comprising the separate operations of applying an agent adapted to inhibit oxidation to selected portions of the material, applying an oxidizing agent, and applying an aromatic compound 45 capable of yielding colourations by oxidation, the oxidation inhibiting agent being applied before at least one of the other agents, and finally effecting formation of said oxidation colourations.

The materials may, for example, be impregnated wholly or in part, for instance by padding or printing, with a solution of a suitable oxidizing agent for example a chlorate or a bichromate, 50 A reducing agent may then be applied locally in

the desired pattern by printing, stencilling, or otherwise, and the material then treated by padding or otherwise with a solution containing a suitable oxidizable aromatic compound or compounds, for example aromatic bases such as p-50 amino-diphenylamine,  $\alpha$ -naphthylamine, benzidine, or aniline. The material is finally subjected to steaming or ageing or other agency to develop the dyeing on those parts to which the oxidizing agent has been applied and has not been 60 rendered inactive by the subsequent application of the reducing agent.

According to another method of carrying the invention into effect the materials may be treated locally in the desired pattern with the reducing agent prior to the application of the oxidizing agent, whereby the latter is rendered ineffective during the subsequent operations of applying and oxidizing the oxidizable aromatic compound.

As reducing agent may be used a hydrosulphite or an oxalate but it is preferred to use one which becomes active on ageing or steaming, for example sodium formaldehyde sulphoxylate, and to dry and age the fabric prior to treatment with 80 the aromatic base or other oxidizable aromatic compound. The material may also be dried between other steps of the process. For application to cellulose ester or ether materials the aromatic amines or other oxidizable compounds 85 may be employed in the form of their soluble salts or in the form of dispersions obtained in any convenient manner and with or without addition of alcohol or other substance having a swelling action on the cellulose derivative. Oxidation catalysts, for example salts of iron, copper, or vanadium, may be used in conjunction 90 with the oxidizing agent, e. g. by incorporation in the solution of the oxidizing agent, or in the solution of the oxidizable aromatic compound 95 or in both. The oxidizing agents and/or reducing agents and/or oxidizable compounds may be applied to the materials in any convenient manner, and if desired or requisite in admixture with thickening agents. A comparatively small 100 quantity of thickener may for example be added to solutions intended for application to the materials by padding but larger quantities may with advantage be added to preparations intended for application by printing.

Coloured "resist" effects may be produced by incorporating in the reducing resist preparation dyestuffs, for example vat-dyestuffs, which are not destroyed thereby and which have affinity for or can be fixed on the material under treatment.

The invention is illustrated, but not limited, by the following examples:—

*Example 1*

5 A fabric woven from cellulose acetate yarns is impregnated in a suitable padding machine with a 5% solution of sodium chlorate and dried. It is then printed with a printing paste of the following composition:—

|    |                                  |       |
|----|----------------------------------|-------|
| 10 |                                  | Grams |
|    | Gum arabic 1:1                   | 600   |
|    | Water                            | 180   |
|    | Caustic soda                     | 20    |
|    | Sodium formaldehyde sulphonylate | 200   |
| 15 |                                  | 1000  |

The printed fabric after drying is padded with the following liquor, being preferably passed direct to the squeezing rollers without previous immersion, the bottom roller running in the liquor.

|    |                        |       |
|----|------------------------|-------|
| 20 |                        | Grams |
|    | Paraaminodiphenylamine | 150   |
|    | Aniline                | 150   |
| 25 | Methylated spirit      | 600   |
|    | Glacial acetic acid    | 450   |
|    | Lactic acid 50%        | 336   |
|    | Cupric chloride        | 14    |
|    | Gum arabic 1:1         | 900   |
| 30 | Water                  | 3600  |
|    |                        | 6200  |

The fabric is now dried and aged in the Mather Platt continuous ager at 100° C. or given other similar suitable steaming after which it is washed well in warm water and finally soaped.

A white pattern on a black ground is obtained. In a similar manner white patterns on a black ground may be produced on materials made of cellulose formate or cellulose propionate.

*Example 2*

45 A fabric woven from cellulose acetate yarns is impregnated with a 5% solution of sodium chlorate and is dried for printing. The chlorate prepared fabric is printed with a paste of the following composition:—

|    |                                  |       |
|----|----------------------------------|-------|
| 50 |                                  | Grams |
|    | Gum arabic 1:1                   | 530   |
|    | Ciba scarlet G                   | 120   |
|    | Caustic soda                     | 10    |
|    | Soda ash                         | 10    |
| 55 | Methylated spirit                | 50    |
|    | Water                            | 150   |
|    | Hydrosulphite                    | 30    |
|    | Sodium formaldehyde sulphonylate | 100   |
| 60 |                                  | 1000  |

The printed fabric is dried and aged in the "rapid ager" at 100° C. or otherwise suitably steamed and then padded, preferably straight through the squeezing rollers, with a pad liquor composed as in Example 1. After drying the material is aged in the "rapid ager" or otherwise suitably steamed, after which it is rinsed lightly and soaped in a soap bath at 60° C. containing 1 gram per litre of sodium perborate till the scar-  
70 let colour is fully developed.

A scarlet pattern on a black ground is obtained.

*Example 3*

A fabric composed of cellulose acetate yarn is 75 impregnated with a 5% solution of sodium di-

|                                  |       |
|----------------------------------|-------|
|                                  | Grams |
| Gum arabic 1:1                   | 600   |
| Water                            | 180   |
| Caustic soda                     | 20    |
| Sodium formaldehyde sulphonylate | 200   |
|                                  | 1000  |

85

The printed fabric after drying is padded with the following liquor, being preferably passed direct to the squeezing rollers without previous immersion, the bottom roller running in the liquor.

|                                   |       |
|-----------------------------------|-------|
| 15                                | Grams |
| Paraphenylenediamine dissolved in | 20    |
| Water                             | 700   |
| Ammonium chloride dissolved in    | 20    |
| Water                             | 50    |
| Sodium formaldehyde sulphonylate  | 1.5   |

95

The padded material after drying is aged in the Mather Platt ager at 100° C. rinsed and finally soaped well.

A white pattern on a brown ground results. 100

*Example 4*

A woven fabric composed of cotton warp and cellulose acetate weft is padded in a 5% solution of sodium chlorate and dried. It is then printed with a printing paste of the following composition:—

|                                |       |
|--------------------------------|-------|
| 20                             | Grams |
| Gum arabic 1:1                 | 260   |
| China clay                     | 100   |
| Zinc formaldehyde sulphonylate | 200   |
| Water                          | 440   |
|                                | 1000  |

115

After drying the printed fabric is given a passage through the "rapid ager" or steamed in the cottage steamer for 3 minutes at 5 lbs. pressure and is then padded, preferably straight through the squeezing rollers with the following padding liquor:—

|                        |       |
|------------------------|-------|
| 30                     | Grams |
| Paraaminodiphenylamine | 150   |
| Aniline                | 150   |
| Methylated spirit      | 600   |
| Glacial acetic acid    | 450   |
| Lactic acid 50%        | 336   |
| Cupric chloride        | 14    |
| Gum tragacanth 5%      | 900   |
| Water                  | 3600  |
|                        | 130   |
|                        | 6200  |

120

The fabric is dried and aged in the "rapid ager" at 100° C. or otherwise suitably steamed, washed in warm water and finally well soaped.

A white pattern on a black ground is obtained.

Though the invention has been more particularly described with reference to the colouring of materials made of or containing cellulose acetate it is also applicable to the colouring of other materials, for example materials made of cotton or a regenerated cellulose type of artificial silk, or of other esters of cellulose, for example cellulose formate, propionate, or butyrate, or the products obtained by the treatment of alkalinized cellulose with esterifying agents (e. g. the product known as "immunized cotton" obtained with p-toluene-sulphochloride), or of cellulose ethers, for instance methyl, ethyl, or benzyl cellulose or the corresponding condensation products of cellulose

135

140

145

150

- and glycols or other polyhydric alcohols, or made of mixtures of two or more of these products.
- What we claim and desire to secure by Letters Patent is:—
5. 1. A process for the production of coloured pattern effects on materials by the formation of oxidation colourations thereon, comprising the separate operations of applying an agent adapted to inhibit oxidation of the color-forming compound to selected portions of the material, of applying an oxidizing agent, and of applying an aromatic compound capable of yielding colourations by oxidation, the oxidation inhibiting agent being applied before at least one of the other agents, and finally effecting formation of said oxidation colourations. 80
2. A process for the production of coloured pattern effects on materials by the formation of oxidation colourations thereon, comprising the separate operations of applying a reducing agent to selected portions of the material, of applying an oxidizing agent, and of applying an aromatic compound capable of yielding colourations by oxidation, the reducing agent being applied before at least one of the other agents, and finally effecting formation of said oxidation colourations. 85
20. 3. A process for the production of coloured pattern effects on materials by the formation of oxidation colourations thereon comprising applying an oxidizing agent, applying a reducing agent locally, applying an aromatic compound capable of yielding colourations by oxidation, and causing the oxidizing agent to effect formation of said oxidation colourations. 90
25. 4. A process for the production of colored pattern effects on materials by the formation of oxidation colorations thereon, comprising applying an oxidizing agent, applying a reducing agent locally, applying an aromatic amine capable of yielding colorations by oxidation, and causing the oxidizing agent to effect formation of said oxidation colorations. 95
30. 5. A process for the production of colored pattern effects on materials, made of or containing cellulose acetate, by the formation of oxidation colorations thereon, comprising applying an oxidizing agent, applying a reducing agent locally in admixture with a coloring matter capable of being fixed on the material, applying an aromatic compound capable of yielding colorations by oxidation, and causing the oxidizing agent to effect formation of said oxidation colorations. 100
35. 6. A process for the production of colored pattern effects on materials made of or containing organic derivatives of cellulose, by the formation of oxidation colorations thereon, comprising the separate operations of applying a reducing agent to selected portions of the material, of applying an oxidizing agent, and of applying an aromatic compound capable of yielding colorations by oxidation, the reducing agent being applied before at least one of the other agents, and finally effecting formation of said oxidation colorations. 105
40. 7. A process for the production of colored pattern effects on materials made of or containing cellulose acetate, by the formation of oxidation colorations thereon, comprising applying an oxidizing agent, applying a reducing agent locally, applying an aromatic compound capable of yielding colorations by oxidation, and causing the oxidizing agent to effect formation of said oxidation colorations. 110
45. 8. A process for the production of colored pattern effects on materials made of or containing cellulose acetate, by the formation of oxidation colorations thereon, comprising applying an oxidizing agent, applying a reducing agent locally, applying an aromatic amine capable of yielding colorations by oxidation, and causing the oxidizing agent to effect formation of said oxidation colorations. 115
50. 9. A process for the production of colored pattern effects on materials made of or containing cellulose acetate, by the formation of oxidation colorations thereon, comprising applying an oxidizing agent, applying a reducing agent locally, applying an aromatic amine capable of yielding colorations by oxidation, and causing the oxidizing agent to effect formation of said oxidation colorations. 120
55. 10. A process for the production of colored pattern effects on materials made of or containing cellulose acetate, by the formation of oxidation colorations thereon, comprising applying an oxidizing agent, applying a reducing agent locally, applying a mixture of aniline and p-amino-diphenylamine, and causing the oxidizing agent to effect formation of said oxidation colorations. 125
60. 11. A process for the production of colored pattern effects on materials made of or containing cellulose acetate, by the formation of oxidation colorations thereon, comprising applying an oxidizing agent, applying a reducing agent locally, applying a mixture of aniline and p-amino-diphenylamine, and causing the oxidizing agent to effect formation of said oxidation colorations. 130
65. GEORGE HOLLAND ELLIS. 135
70. WILLIAM BERTRAM MILLER. 140
75. 145
80. 150